

Patented Apr. 5, 1927.

1,623,085

# UNITED STATES PATENT OFFICE.

AMANDUS BARTELS AND OTTO MIECH, OF HARBURG-ON-THE-ELBE, GERMANY.

## MANUFACTURE OF SHAPED ARTICLES OF CASEIN.

No Drawing. Application filed March 24, 1926, Serial No. 97,141, and in Germany May 15, 1923.

The usual method of manufacturing shaped articles from artificial horn made of casein consists in obtaining roughly formed pieces from already hardened bars 5 or plates by cutting, stamping or in some other manner, which are thereupon heated up to about 100° in an oil bath or some other suitable way and given their finished form by pressing. The disadvantages of this 10 method are the very laborious and costly operations involved, the difficulty of utilizing the waste often produced in large quantities and the danger of the finished articles becoming deformed when in use, for instance 15 owing to the action of moisture. It has already been proposed to produce shaped articles in a similar manner to the way bars and plates have hitherto been produced, viz, by first pressing the casein material and 20 thereupon to harden and dry the articles so formed. But this method has not been adopted in practice in the art for the production of the actual shaped articles, as the 25 shaped articles become deformed during the hardening and drying operation, and it is not possible by subsequent treatment to obtain articles that will really keep their shape when in use.

According to the new method shaped 30 articles may be successfully produced from the casein material before it is hardened or after it has been treated only with weak hardening agents, which by subsequent hardening and drying give products which 35 keep their form well. This is effected by using for the manufacture of the shaped articles separate pieces of a relatively dry casein material containing about 20% or slightly less water. The separate pieces of 40 a suitable size and form and a content of water amounting preferably to between 12 and 16% are softened by the action of heat for instance in a current of hot air, in steam, a hot liquid which has no detrimental action 45 on the casein material or by means of any suitable heating device, given their final form, hardened, dried and if necessary, subsequently operated upon. The casein material which is treated in this way, may be 50 obtained from slightly moistened casein or a casein mixture, for instance by kneading under high pressure, the water content being so small as not to exceed 20%. This relatively dry material may be used directly in 55 the form of pieces cut from the extruded

length for the manufacture of buttons, counters and the like. According to the present invention the pieces cut from the extruded length or formed in some other way may be preliminarily dried, until they are 60 about as dry as the surrounding air, that is contain from 10 to 14% of water. On the other hand the casein material obtained by any process and having any water content may be used for the separate and preliminarily formed pieces after being subjected to 65 a preliminary drying operation until the water content is 20% or less, so that they are approximately as dry as the surrounding air.

The new process, in which the manufacture of the artificial horn from casein and of the finished articles of all kinds from the same are completely combined, is particularly suitable for the manufacture on a large 70 scale of handles, buttons, toy building bricks, rings, ornaments, bars of different shape and size and the like. It is a special advantage of the new process that the formed pieces are hardened much more rapidly. When 75 working up the moistened casein or casein mixture to form the mass agents having a slight hardening action may be added. The articles formed from this mass need only be immersed for a short time in an effective 80 hardening bath, for instance, a solution of formaldehyde, it being only necessary for the superficial layer to be subsequently hardened for ensuring that the articles will 85 retain their shape.

For giving them a preliminary hardening the separate pieces may first be immersed in a bath having a weak action and consisting for instance of solutions of aluminum salts or other metal salts having a hardening 90 action on casein, of tannic acids or other acids having such a hardening action, but preferably in a bath of formaldehyde compounds having a slight hardening action, for instance hexamethylentetramin, until 95 they are hardened right through. The separate pieces even after being dried in this manner may be softened and successfully pressed and stamped. Through this preliminary and subsequent hardening of the 100 surface layer, the time taken for the hardening operation is considerably reduced and still the form obtained by pressing will be such that any subsequent deformation of the pressed articles, such as would take place 110

if the ordinary casein mass were made directly into shaped articles cannot possibly occur.

Having now particularly described and ascertained the nature of our said invention and in what manner the same is to be performed, we declare that what we claim is:

1. A method of manufacturing shaped articles from artificial horn made from casein, consisting in producing from non-hardened casein material separate pieces corresponding in size and shape to the desired product, with such material containing approximately between 7 and 17% of water, rapidly softening such pieces by the action of heat, treating such pieces to give them their final form, and finally hardening and drying the pieces.
2. A method of manufacturing shaped articles from artificial horn made from casein, consisting in producing from non-hardened casein material separate pieces corresponding in size and shape to the desired product, with such material containing approximately between 7 and 17% of water, rapidly softening such pieces by the action of moist heat, treating such pieces to give them their final form, and finally hardening and drying the pieces.
3. A method of manufacturing shaped articles from artificial horn made from casein consisting in producing separate pieces of the size and shape of the final product, preliminarily treating such pieces by a weak hardening agent, drying such pieces until

they contain a suitable water content approximating 17%, softening the pieces under the action of heat and finally shaping the pieces so softened into their required final form.

4. A method of manufacturing shaped articles from artificial horn made from casein consisting in producing separate pieces of the size and shape of the final product, preliminarily treating such pieces by a weak hardening agent, drying such pieces until they contain a suitable water content approximating 17%, softening the pieces under the action of heat and finally shaping the pieces so softened into their required final form, and thereafter treating the formed pieces to harden their superficial layer.

5. A method of manufacturing shaped articles from artificial horn made from casein consisting in dividing the casein mass into pieces corresponding to the size and shape of the final product, treating the pieces in a bath having a weak hardening action, drying the pieces to a limit of approximately 17% water content, softening the pieces by the action of heat, giving the pieces their final form under pressure, and subjecting the formed pieces to the action of a hardening agent until the superficial layer of each piece is hardened, and finally drying the pieces.

In testimony whereof we affix our signatures.

DR. AMANDUS BARTELS.  
OTTO MIECH.